

## UNITED STATES PATENT OFFICE

2,185,617

## HIGH-SPEED STEEL

Elmer B. Welch, McKeesport, and Lewis Gerald Firth, Pittsburgh, Pa., assignors to Firth-Sterling Steel Company, a corporation of Pennsylvania

No Drawing. Application May 24, 1939,  
Serial No. 275,466

## 6 Claims. (Cl. 75—123)

This invention relates to high-speed steel of molybdenum type.

In an application for Letters Patent, filed January 21, 1939, Serial No. 252,214, we have disclosed the discovery that boron may advantageously be included in the mix for steel of this type. It is our discovery that, boron being present in an amount that, in the twenty examples there given, ranges from 0.10 to 0.91% of the iron content, chromium may be entirely eliminated; and that if chromium be eliminated or (being present) is present in quantity not exceeding 1.50% of the iron content, a steel is produced that is free of any tendency to deteriorate in heat-treatment, and a steel that possesses the desirable qualities characteristic of the type.

Our present invention relates to the same subject-matter and, more specifically, to the inclusion in the mix of cobalt, either with or without nickel also.

In accordance with this invention, an alloy may contain the following elements within the percentages given (the percentages being relative to the iron content)—

|            |            |
|------------|------------|
| Carbon     | .30-1.10   |
| Silicon    | .05-1.00   |
| Manganese  | .10-1.00   |
| Vanadium   | .25-2.50   |
| Molybdenum | 5.00-12.00 |
| Cobalt     | .50-15.00  |
| Boron      | .05-.50    |

It may additionally contain chromium, if the chromium content does not exceed 1.50 percent of the iron; and, in addition to cobalt, it may contain (and advantageously contain) nickel, in an amount ranging upward to 5 percent.

Several varieties or specific examples of cobalt types of alloy compositions falling within the above given ranges of percentages for the various ingredients, arranged in the order of their cobalt content are as follows:

| No.  | C   | Si  | Mn  | Cr   | Va   | Mo    | Co    | Ni   | B   |
|------|-----|-----|-----|------|------|-------|-------|------|-----|
| I    | .42 | .76 | .47 | 1.06 | .25  | 6.18  | 1.06  | 4.01 | .43 |
| II   | .51 | .43 | .82 | .81  | .46  | 8.60  | 2.62  | —    | .29 |
| III  | .62 | .57 | .51 | .93  | .92  | 5.82  | 3.51  | 1.55 | .37 |
| IV   | .63 | .33 | .27 | .76  | .80  | 8.27  | 5.17  | —    | .22 |
| V    | .68 | .38 | .18 | 1.20 | 1.25 | 10.58 | 7.03  | .47  | .14 |
| VI   | .81 | .46 | .32 | .88  | 1.83 | 13.01 | 8.89  | —    | .27 |
| VII  | .79 | .29 | .37 | .09  | 2.05 | 9.26  | 11.92 | —    | .23 |
| VIII | .73 | .16 | .39 | 1.03 | 1.62 | 8.43  | 14.01 | —    | .19 |

The remainder of the compositions tabulated above will be understood to be substantially of

iron, together with such other alloying elements and impurities as are sometimes found in this type of alloy compositions.

The above examples all contain cobalt. Some contain cobalt and nickel also. Their hardening temperatures range from about 1800° F. to 2350° F. The range of drawing temperatures, at which secondary hardness is developed is from 900° to 1200° F. The effect of the presence of cobalt (and cobalt and nickel) is that the ranges both of hardening and of tempering temperatures (at which full hardness and strength may be developed) are broadened. The addition also increases somewhat the maximum attainable hardness and increases the resistance of the steel to tempering.

The steel of the present invention is particularly suitable for dies and for high-speed cutting tools.

If the steel is to be used for dies, a composition such as the following may be used (again, percentages are given with reference to the iron content):

|            | Effective composition | Preferred composition |
|------------|-----------------------|-----------------------|
| Carbon     | .30-.65               | .40-.60               |
| Silicon    | .15-1.00              | .35-.80               |
| Manganese  | .15-1.00              | .30-.65               |
| Chromium   | .00-1.50              | .15-.50               |
| Vanadium   | .00-2.50              | .25-1.25              |
| Molybdenum | 5.00-12.00            | 6.00-11.00            |
| Cobalt     | .50-10.00             | 1.00-6.00             |
| Nickel     | .00-5.00              | .25-2.00              |
| Boron      | .15-.50               | .15-.40               |

If the steel is to be used as a cutting tool a composition such as the following may be used:

|            | Effective composition | Preferred composition |
|------------|-----------------------|-----------------------|
| Carbon     | .50-1.10              | .50-1.10              |
| Silicon    | .00-1.00              | .10-1.00              |
| Manganese  | .00-1.00              | .10-1.00              |
| Chromium   | .00-1.25              | .00-1.50              |
| Vanadium   | .00-2.50              | .25-2.50              |
| Molybdenum | 5.00-12.00            | 5.00-12.00            |
| Cobalt     | .50-15.00             | 1.00-15.00            |
| Nickel     | .00-5.00              | .00-2.50              |
| Boron      | .05-.50               | .05-.50               |

Dies which proved effective were found upon analysis to contain—

| O   | Si  | Mn  | Cr   | Va  | Mo   | Co   | Ni   | B   |
|-----|-----|-----|------|-----|------|------|------|-----|
| .42 | .76 | .47 | 1.06 | .25 | 6.18 | 1.06 | 4.01 | .43 |

Another steel which also gave highly satisfac-

5 tory results as a steel for dies and also proved superior to 18-4-1 steel as a cutting tool—

| 5 | C   | Si  | Mn  | Cr  | Va  | Mo   | Co   | Ni    | B   |
|---|-----|-----|-----|-----|-----|------|------|-------|-----|
|   | .51 | .43 | .82 | .31 | .46 | 8.60 | 2.62 | ..... | .29 |

10 Still better steel for dies may contain—

| 10 | C   | Si  | Mn  | Cr  | Va  | Mo   | Co   | Ni   | B   |
|----|-----|-----|-----|-----|-----|------|------|------|-----|
|    | .62 | .57 | .51 | .93 | .92 | 5.82 | 3.51 | 1.52 | .37 |

15 15 A tool steel alloyed in accordance with the invention which in service test was found superior to 18-4-1 and other known types of molybdenum high-speed steels was found upon analysis to contain—

| 20 | C   | Si  | Mn  | Cr  | Va  | Mo   | Co   | Ni    | B   |
|----|-----|-----|-----|-----|-----|------|------|-------|-----|
|    | .63 | .33 | .27 | .76 | .89 | 8.27 | 5.17 | ..... | .22 |

25 Still better tool steels were found to contain—

| 30 | C   | Si  | Mn  | Cr   | Va   | Mo    | Co    | Ni    | B   |
|----|-----|-----|-----|------|------|-------|-------|-------|-----|
|    | .68 | .38 | .18 | 1.20 | 1.25 | 10.58 | 7.03  | .47   | .14 |
|    | .81 | .46 | .32 | .88  | 1.83 | 13.01 | 8.50  | ..... | .27 |
|    | .79 | .29 | .37 | .09  | 2.05 | 9.26  | 11.92 | ..... | .23 |
|    | .73 | .16 | .39 | 1.03 | 1.62 | 8.43  | 14.01 | ..... | .19 |

35 Cobalt when added to a steel in which boron is present and from which chromium is either wholly eliminated or, being present, does not exceed 1.50% of the iron content, increases red-hardness, affords greater toughness, and improves the cutting quality. If, additionally, nickel also be present, higher temperature in 40 heat-treatment is gained, and the good qualities just specified are realized in yet larger measure.

45 We have specified that the steel of our invention may be free of chromium; and that, if chromium be present, it should not exceed in quantity 1.50 percent of the iron content. We characterize such a steel as substantially free of chromium.

We claim as our invention:

50 1. A high-speed steel of molybdenum type, substantially free of chromium, whose other non-ferrous components, in percentages relative to the iron content, are—

| 55 | Carbon     | Percent    |
|----|------------|------------|
|    | Carbon     | 0.30- 1.10 |
|    | Silicon    | 0.05- 1.00 |
|    | Manganese  | 0.10- 1.00 |
|    | Vanadium   | 0.25- 2.50 |
|    | Molybdenum | 5.00-12.00 |
|    | Boron      | 0.05- 0.50 |

60 together with metal of a group that consists of cobalt and nickel, in quantity ranging from 0.50 to 20 percent.

65 2. A high-speed steel of molybdenum type, substantially free of chromium, whose other non-

ferrous components, in percentages relative to the iron content, are—

|            | Percent    |
|------------|------------|
| Carbon     | 0.30- 1.10 |
| Silicon    | 0.50- 1.00 |
| Manganese  | 0.10- 1.00 |
| Vanadium   | 0.25- 2.50 |
| Molybdenum | 5.00-12.00 |
| Cobalt     | 0.50-15.00 |
| Nickel     | Up to 5.00 |
| Boron      | 0.05- 0.50 |

70 3. A high-speed steel of molybdenum type, substantially free of chromium, whose non-ferrous components, in percentages relative to the iron content, are—

|            | Percent    |
|------------|------------|
| Carbon     | 0.40- 0.60 |
| Silicon    | 0.35- 0.80 |
| Manganese  | 0.30- 0.65 |
| Vanadium   | 0.25- 1.25 |
| Molybdenum | 6.00-11.00 |
| Cobalt     | 1.00- 6.00 |
| Nickel     | 0.25- 2.00 |
| Boron      | 0.15- 0.40 |

75 4. A high-speed steel of molybdenum type, substantially free of chromium, whose non-ferrous components, in percentages relative to the iron content, are—

|            | Percent    |
|------------|------------|
| Carbon     | 0.50- 1.10 |
| Silicon    | 0.10- 1.00 |
| Manganese  | 0.10- 1.00 |
| Vanadium   | 0.25- 2.50 |
| Molybdenum | 5.00-12.00 |
| Boron      | 0.05- 0.50 |

80 together with metal of a group that consists of cobalt and nickel, in quantity ranging from 1.00 to 17.50 percent.

85 5. A high-speed steel of molybdenum type, substantially free of chromium, and of the following composition, the quantities of the non-ferrous components being given in percentage relative to the iron component: carbon, 0.62 percent; silicon, 0.57; manganese, 0.51; vanadium, 0.92; molybdenum, 5.82; cobalt, 3.51; nickel, 1.52; boron, 0.37, the residue being substantially of iron.

90 6. A high-speed steel of molybdenum type, substantially free of chromium, whose non-ferrous components, in percentages relative to the iron content, are—

|            | Percent    |
|------------|------------|
| Carbon     | 0.68- 0.81 |
| Silicon    | 0.16- 0.46 |
| Manganese  | 0.18- 0.39 |
| Vanadium   | 1.25- 2.05 |
| Molybdenum | 8.43-13.01 |
| Boron      | 0.14- 0.27 |

95 together with metal of a group that consists of cobalt and nickel, in quantity ranging from 7.03 to 14.48 percent.

ELMER B. WELCH.  
LEWIS GERALD FIRTH.